

## UNITED STATES PATENT OFFICE

2,490,745

CELLULOSE CARBOXYLIC ESTER SILVER  
HALIDE EMULSIONS SENSITIZED WITH  
BENZOTHIAZOLE AND BENZOLENA-  
ZOLE QUATERNARY SALTSBurt H. Carroll and William West, Rochester,  
N. Y., assignors to Eastman Kodak Company,  
Rochester, N. Y., a corporation of New JerseyNo Drawing. Application January 13, 1948,  
Serial No. 2,126

13 Claims. (Cl. 95—7)

1

This invention relates to sensitized photographic emulsions and more particularly to cellulose carboxylic ester silver halide photographic emulsions sensitized with benzothiazole and benzoselenazole quaternary salts.

It is known that benzothiazole, benzoselenazole, benzoxazole, naphthothiazole, simple thiazole and thiazoline quaternary salts when incorporated in gelatino-silver-halide emulsions for example in a concentration of from 2 to 8 mg. per 100 cc. of emulsion, act as antifoggants for the emulsions. (See United States Patent 2,131,038, dated September 27, 1938.) It is also known that pyridinium and quinolinium quaternary salts act to supersensitize cyanine dyes in photographic silver halide emulsions. (See United States Patent 2,334,864, dated November 23, 1943.) It is also known that surface active quaternary ammonium salts sensitize photographic silver halide emulsions. (See United States Patent 2,271,623, dated February 3, 1942.)

We have now found that substantially non-surface active quaternary salts of the benzothiazole and benzoselenazole series sensitize cellulose carboxylic ester silver halide emulsions, although these same quaternary salts act as antifoggants in gelatino-silver-halide emulsions. Moreover, we have found that substantially non-surface active quaternary salts of simple thiazoles, naphthothiazoles and tetrahydrobenzothiazoles do not sensitize cellulose carboxylic ester silver halide emulsions.

It is an object of our invention, therefore, to provide sensitized cellulose carboxylic ester silver halide emulsions. A further object is to provide a process for preparing such emulsions. Other objects will become apparent hereinafter.

The quaternary salts which we employ in practicing our invention are substantially colorless, substantially non-surface active quaternary salts of the benzothiazole and of the benzoselenazole series, which are devoid of nitro groups. A preferred group of these quaternary salts are represented by the following general formula:



wherein D represents an o-arylene group of the benzene series containing from 6 to 8 carbon atoms and which is devoid of nitro groups; e. g. the o-phenylene group, a chloro-o-phenylene group,

group, a methyl-o-phenylene group, a methoxy-o-phenylene group, a bromo-o-phenylene group, an ethoxy-o-phenylene group, an ethyl-o-phenylene group, a dimethyl-o-phenylene group, etc., 5 Q represents a sulfur atom or a selenium atom, R represents a primary alkyl group containing from 1 to 4 carbon atoms, i. e. methyl, ethyl, n-propyl, isobutyl and n-butyl, a primary alkenyl group containing from 3 to 4 carbon atoms, i. e. allyl, 2-butenyl and 3-butenyl, a primary hydroxyalkyl group containing from 2 to 4 carbon atoms, i. e.  $\beta$ -hydroxyethyl,  $\gamma$ -hydroxypropyl,  $\beta$ -hydroxypropyl,  $\delta$ -hydroxybutyl,  $\gamma$ -hydroxybutyl and  $\beta$ -hydroxybutyl, a primary alkoxyalkyl group, containing from 3 to 4 carbon atoms, e. g.  $\beta$ -methoxyethyl,  $\beta$ -ethoxyethyl,  $\beta$ -methoxypropyl and  $\gamma$ -methoxypropyl, R<sub>1</sub> represents a hydrogen atom, a methyl group, an ethyl group, an alkylmercapto group containing from 1 to 4 carbon atoms, e. g. methylmercapto, ethylmercapto, n-propylmercapto, n-butylmercapto, isobutylmercapto, an arylmercapto group containing from 6 to 8 carbon atoms and devoid of nitro groups, e. g. phenylmercapto, p-tolylmercapto, 10 p-chlorophenylmercapto, etc., a primary amino group (i. e. —NH<sub>2</sub>), an alkylamino group containing from 1 to 4 carbon atoms, e. g. methylamino, ethylamino, n-propylamino, n-butylamino, etc., a dialkylamino group containing from 2 to 4 carbon atoms, e. g. dimethylamino, diethylamino, etc., an arylamino group containing from 6 to 8 carbon atoms and devoid of nitro groups, e. g. phenylamino,  $\beta$ -tolylamino, p-chlorophenylamino, p-methoxyphenylamino, N-methyl-N-phenylamino, etc., or an aralkylamino group containing from 6 to 8 carbon atoms, and devoid of nitro groups, e. g. N-methyl-N-benzylamino, benzylamino,  $\beta$ -phenylethylamino, etc., and X represents an anion, e. g. chloride, bromide, iodide, methylsulfate, ethylsulfate, p-toluenesulfonate, benzenesulfonate, perchlorate, acetate, propionate, n-butyrate, thiocyanate, sulfamate, etc., 15 20 25 30 35 40 45 50 55 60 65 70 75 80 85 90 95 100 Examples of the above-formulated quaternary salts which are especially useful are: benzothiazole ethiodide, benzothiazole metho-p-toluenesulfonate, 2-methylbenzothiazole metho-p-toluene-sulfonate, 2-methylbenzothiazole etho-p-toluenesulfonate, 2-methylbenzothiazole alliodide, 2-methylbenzothiazole n-butiodide, 5-chloro-2-methylbenzothiazole etho-p-toluenesulfonate, 2-methylmercaptobenzothiazole metho-p-toluenesulfonate, 2-phenylmercaptobenzothiazole ethiodide, 2-anilinobenzothiazole ethiodide, 2-

methylbenzoselenazole ethiodide, 5-chloro-2-methylbenzoselenazole ethiodide, 2-methylbenzothiazole  $\beta$ -hydroxyethobromide, etc.

The effect of these quaternary salts of the benzothiazole and of the benzoselenazole series in cellulose carboxylic ester silver halide emulsions is to increase the speed of the emulsions. The speed increase may be accompanied by a loss in contrast. In the case of cellulose carboxylic ester silver halide emulsions which are optically sensitized by the addition of a sensitizing dye, the increase in speed is approximately the same in the color-sensitized and non-color-sensitized regions of spectral sensitivity. Benzothiazole methiodide or metho-p-toluenesulfonate effect a large speed increase, but with a considerable lowering of contrast. 2-methylbenzothiazole etho-p-toluene-sulfonate is very active in increasing speed, without reducing contrast as much as the unsubstituted benzothiazole quaternary salt. 2-methyl-mercaptopbenzothiazole metho-p-toluenesulfonate and 2-phenylmercaptopbenzothiazole ethiodide are very active.

To sensitize cellulose carboxylic ester silver halide emulsions with these quaternary salts, it is only necessary to disperse the quaternary salts in the emulsion. It is convenient to add the quaternary salts to the emulsions from solutions in appropriate solvents. Water, methyl alcohol or ethyl alcohol or mixtures of these three solvents are suitable. The concentration of the quaternary salts in the emulsion can vary widely. Usually the optimum sensitizing effect is obtained at from 0.01 to 0.05 gram per liter of emulsion. However, higher or lower concentrations can be used. The quaternary salts can be added to the emulsion at any stage of its preparation, but are most advantageously added to the finished emulsions just prior to coating the

for the quaternary salts. The concentration of the sensitizing dye can vary widely, e. g. from 5 to 100 mg. per liter of emulsion. Ordinarily from 10 to 50 mg. of dye per liter of emulsion suffices to produce optimum optical sensitization. Both the sensitizing dyes and the quaternary salts should be thoroughly dispersed throughout the emulsions by stirring or other means.

As cellulose carboxylic ester silver halide emulsions those described in United States Patent 2,110,491, dated March 8, 1931, in United States Patent 2,276,322, dated March 17, 1942, and in United States Patent 2,127,573, dated August 23, 1938, are examples. Photographic silver halide emulsions prepared using as vehicle or carrier hydrolyzed cellulose carboxylic esters, such as hydrolyzed cellulose acetate or hydrolyzed cellulose acetate propionate containing from 19 to 33 per cent by weight of acyl groups are especially useful in practicing our invention. Those containing 20 to 26 per cent by weight of acyl groups are most advantageously employed. Any cellulose compound especially those containing only carbon, hydrogen, oxygen and amino nitrogen atoms, or ammonium nitrogen atoms, which are soluble in a mixture of ethyl alcohol and water (containing from 0 to 50 per cent by volume of ethyl alcohol) to the extent of 10 g. per 100 g. of solvent can be employed as the vehicle or carrier for the silver halide. The silver halides can be silver chloride, silver bromide, silver iodide or mixtures of one or more of these silver halides, for example.

The following table illustrates results which can be obtained in accordance with our invention. The emulsion employed was a hydrolyzed cellulose acetate silver chlorobromoiode emulsion in which the cellulose acetate contained from 23 to 24 per cent by weight of acetyl groups.

Table

|     | Quaternary Salt                                            | Gms. per liter of emulsion | Speed       |                                |                         | Gradient    |                   |      |
|-----|------------------------------------------------------------|----------------------------|-------------|--------------------------------|-------------------------|-------------|-------------------|------|
|     |                                                            |                            | Total Light | Total, Minus Blue <sup>1</sup> | Blue Light <sup>2</sup> | Total Light | Total, Minus Blue | Blue |
| (a) | None                                                       |                            | 3,610       | -----                          | 202                     | 1.00        | -----             | 1.22 |
| (b) | Benzothiazole methiodide                                   | 0.025                      | 5,890       | -----                          | 372                     | 1.10        | -----             | 1.19 |
| (c) | None <sup>3</sup>                                          |                            | 7,230       | 2,880                          | 275                     | 1.54        | 1.42              | 1.32 |
| (d) | Benzothiazole methiodide                                   | 0.013                      | 9,800       | 4,680                          | 468                     | 1.42        | 1.05              | 1.27 |
| (e) | do                                                         | 0.050                      | 14,400      | 5,600                          | 455                     | 1.04        | 1.07              | 0.97 |
| (f) | Benzothiazole metho-p-toluene-sulfonate                    | 0.025                      | 10,200      | 5,300                          | 478                     | 0.98        | 1.38              | 1.21 |
| (g) | None <sup>3</sup>                                          |                            | 2,950       | 950                            | 169                     | 1.41        | 1.50              | 1.36 |
| (h) | 2-Methylbenzo-thiazole metho-p-toluene-sulfonate           | 0.025                      | 4,780       | 1,480                          | 282                     | 1.31        | 1.38              | 1.12 |
| (i) | do                                                         | 0.050                      | 5,610       | 1,940                          | 331                     | 1.15        | 1.27              | 1.12 |
| (j) | 2-Methylbenzo-thiazole etho-p-toluene-sulfonate            | 0.025                      | 4,660       | 1,660                          | 245                     | 1.46        | 1.48              | 1.30 |
| (k) | None <sup>3</sup>                                          |                            | 3,160       | 1,200                          | 123                     | 1.62        | 1.62              | 1.62 |
| (l) | 2-Methyl-mercaptopbenzo-thiazole metho-p-toluene-sulfonate | 0.025                      | 4,160       | -----                          | 174                     | 1.50        | -----             | 1.58 |
| (m) | 2-Phenylmercaptopbenzothiazole ethiodide                   | 0.025                      | 7,230       | 2,950                          | 324                     | 1.34        | 1.25              | 1.20 |

<sup>1</sup> Total-minus-blue speed was measured through a filter which transmitted substantially no light of wavelength shorter than 300  $\mu$ .

<sup>2</sup> Blue light speed was measured through a filter which transmitted substantially no light except between 360 and 500  $\mu$ .

<sup>3</sup> 2,3'-diethyl-4'-methylxantholocarbocyanine iodide used in the emulsion in a concentration of 20 mg. per liter of emulsion, as color-sensitizer.

emulsions. One or more of the quaternary salts can be employed.

The quaternary salts can be employed in conjunction with sensitizing dyes and the quaternary salts can be added to the emulsion before, after or simultaneously with the sensitizing dyes. One or more sensitizing dyes can be used. The sensitizing dyes can be added to the emulsions in the usual manner from a solution in an appropriate solvent, e. g. the solvents set forth above

Various kinds of sensitizing dyes can be employed in connection with the quaternary salts, e. g. cyanine dyes, merocyanine dyes, hemicyanine dyes, hemioxonol dyes, styrl dyes, etc. Sensitizing dyes of these kinds are described and defined for example in "The Theory of the Photographic Process" by C. E. K. Mees, The Macmillan Company, New York, 1942. Merocyanine dyes are also described by L. G. S. Brooker in 75 United States Patent 2,170,803, dated August 29,

1939 and in United States Patent 2,078,233, dated April 27, 1937. Hemicyanine dyes are described by F. L. White and G. H. Keyes in United States Patent 2,263,749, dated November 25, 1941. Hemioxonol dyes are described by G. H. Keyes in United States Patent 2,186,608, dated January 9, 1940.

The quaternary salts which we employ in practicing our invention for the most part can be prepared from the corresponding benzothiazole or benzoselenazole bases by heating the heterocyclic base with the appropriate alkyl salt, using a closed tube where higher temperatures are desired or the volatility of the reactants demands. Methods for preparing hydroxyalkyl, alkoxyalkyl and other substituted alkyl quaternary salts are described in United States Patents 2,231,658, dated February 11, 1941 and 2,213,238, dated September 3, 1940. Alkylmercaptobenzothiazoles and alkylmercaptobenzoselenazoles can be prepared by alkylating the corresponding mercapto compounds. The resulting alkylmercapto benzothiazoles and benzoselenazoles can then be quaternarized by heating with an alkyl salt. 2-arylmercaptobenzothiazoles can be prepared from 2-chlorobenzothiazoles by treating the 2-chlorobenzothiazoles with an aryl mercaptan, in the presence of triethylamine (Brooker et al., Jour. Am. Chem. Soc. 63, 3200 (1941)). The arylmercaptobenzothiazoles can then be quaternarized by heating with alkyl salts (Brooker et al., supra). 2-arylmercaptobenzoselenazoles can be prepared in the same manner. 2-chlorobenzoselenazole can be prepared as described by Hasan et al. Jour. Chem. Soc. (London) 1935, 1762. 2-arylaminobenzothiazole quaternary salts can be prepared by condensing 2-phenylmercaptobenzothiazole quaternary salts with a primary aromatic amine or a N-alkyl aromatic amine (Brooker et al., supra). Instead of 2-phenylmercaptobenzothiazole quaternary salts, 2-ethylmercaptobenzothiazole quaternary salts can be used. 2-alkylamino-, 2-dialkylamino- and 2-aralkylaminobenzothiazole quaternary salts can be similarly prepared using a primary aliphatic amine, a secondary aliphatic amine or an aralkylamine instead of the aryl amine. 2-amino-, 2-methylamino- and 2-anilinobenzoselenazole are described by Hasan et al., supra. Starting with 2-ethylmercaptobenzoselenazole quaternary salts, 2-arylmino-2-aralkylamino- and 2-alkylamino-benzoselenazole quaternary salts can be prepared as described above for the corresponding benzothiazole compounds. 2-aminobenzothiazole quaternary salts can be prepared by adding hydrogen chloride to 3-alkyl-2-iminobenzothiazoline. 2-aminobenzoselenazole quaternary salts can be similarly prepared from 3-alkyl-2-iminobenzoselenazolines (described by Hasan et al., supra). The chloride anion of any of these quaternary chlorides can be converted to the bromide or iodide anion by treating an aqueous or methyl or ethyl alcoholic solution of the quaternary chloride with an aqueous solution of potassium bromide or iodide. The quaternary chlorides, bromides or iodides can be converted to quaternary perchlorates by treating a hot alcoholic solution of the quaternary halide with an aqueous solution of sodium perchlorate. Quaternary iodides can be converted to quaternary chlorides, quaternary acetates or quaternary thiocyanates by heating the quaternary iodide with a suspension of silver chloride, silver acetate or silver thiocyanate in methyl alcohol. Similar conversions of quaternary iodides to quaternary

chlorides can be made by heating the quaternary iodide with silver chloride in a phenol. (See United States Patent 2,245,249, dated June 10, 1941.)

5 The 2-methylbenzothiazole bases from which 2-methylbenzothiazole quaternary salts can be prepared by heating with an alkyl salt, are for the most part preparable by the method of Fries et al., Ann 407, 208 (1915) in which the appropriate thioacetylaniline is oxidized with alkaline potassium ferricyanide. Thus, p-chlorothioacetanilide gives 6-chloro-2-methylbenzothiazole. The thioacetylanilines can be prepared by treating the corresponding acetylaniline with phosphorus pentasulfide in dry benzene or xylenes. The acetylanilines can be prepared by the action of acetic anhydride or acetyl chloride on the corresponding aniline compound. Several of the 2-methylbenzothiazole bases can also be prepared by reducing bis(o-nitrophenyl) disulfides with zinc dust and acetic acid, acetyloyating the reduction mixture with acetic anhydride and closing the ring by heating the resulting mixture. The bis(o-nitrophenyl) disulfides can be prepared from the corresponding o-bromonitrobenzenes by heating the o-bromonitrobenzene with sodium disulfide in methyl alcohol. Thus, 2-bromo-4-chloronitrobenzene gives bis(5-chloro-2-nitrophenyl) disulfide which, on reduction, acetylation of the reduction product and heating gives 2-methyl-6-chlorobenzothiazole. 2-methylbenzoselenazole bases can be prepared by reducing bis(o-nitrophenyl) diselenides with zinc dust and acetic acid, acetyloyating the reaction mixture with acetic anhydride, and closing the ring by heating the resulting mixture. The bis(o-nitrophenyl) diselenides can be prepared from the corresponding o-bromonitrobenzenes by heating the o-bromonitrobenzenes with sodium selenide in methyl alcohol. See also Clark, J. Chem. Soc. (London), 1928, 2313.

What we claim as our invention and desire to be secured by Letters Patent of the United States is:

1. A photographic silver halide emulsion in which the silver halide is dispersed in a hydrolyzed cellulose carboxylic ester containing from 19 per cent to 33 per cent by weight of acyl groups, said emulsion being sensitized with at least one quaternary salt selected from the group of quaternary salts represented by the following general formula:



55 wherein D represents an o-arylene group of the benzene series containing from 6 to 8 carbon atoms and which is devoid of nitro groups, Q represents a member selected from the group consisting of a sulfur atom and a selenium atom, R represents a member selected from the group consisting of a primary alkyl group containing from 1 to 4 carbon atoms, a primary alkenyl group containing from 3 to 4 carbon atoms, a primary hydroxyalkyl group containing from 2 to 4 carbon atoms, and a primary alkoxyalkyl group containing from 3 to 4 carbon atoms, R<sub>1</sub> represents a member selected from the group consisting of a hydrogen atom, a methyl group, an ethyl group, an alkyl mercapto group containing from 1 to 4 carbon atoms, an arylmercapto group containing from 6 to 8 carbon atoms and which is devoid of nitro groups, a primary amino group, an alkyl amino group containing from 1 to 4 carbon

atoms, a dialkylamino group containing from 2 to 4 carbon atoms, an arylamino group containing from 6 to 8 carbon atoms and which is devoid of nitro groups and an aralkylamino group containing from 6 to 8 carbon atoms and which is devoid of nitro groups, and X represents an anion.

2. A photographic silver halide emulsion in which the silver halide is dispersed in a hydrolyzed cellulose carboxylic ester containing from 19 per cent to 33 per cent by weight of acyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, and X represents an anion.

3. A photographic silver halide emulsion in which the silver halide is dispersed in a hydrolyzed cellulose acetate containing from 19 per cent to 33 per cent by weight of acetyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, and X represents an anion.

4. A photographic silver halide emulsion in which the silver halide is dispersed in a hydrolyzed cellulose acetate containing from 20 per cent to 26 per cent by weight of acetyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, and X represents an anion.

5. A photographic silver halide emulsion in which the silver halide is dispersed in a hydrolyzed cellulose carboxylic ester containing from 19 per cent to 33 per cent by weight of acyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, R1 represents an alkylmercapto group containing from 1 to 4 carbon atoms, and X represents an anion.

6. A photographic silver halide emulsion in which the silver halide is dispersed in a hydrolyzed cellulose acetate containing from 19 to 33 per cent by weight of acetyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, R1 represents an alkylmercapto group containing from 1 to 4 carbon atoms, and X represents an anion.

7. A photographic silver halide emulsion in which the silver halide is dispersed in a hydrolyzed cellulose acetate containing from 20 to 26 per cent by weight of acetyl groups, said emulsion being sensitized with at least one quaternary salt selected from the group consisting of those quaternary salts represented by the following general formula:



wherein D represents an o-arylene group of the benzene series containing from 6 to 8 carbon atoms and which is devoid of nitro groups, R represents a primary alkyl group containing from 1 to 4 carbon atoms, R1 represents an alkylmercapto group containing from 1 to 4 carbon atoms, and X represents an anion.

8. A photographic silver halide emulsion in which the silver halide is dispersed in a hydrolyzed cellulose acetate containing from 20 to 26 per cent by weight of acetyl groups, said emulsion being sensitized with 2-methylbenzothiazole etho-p-toluenesulfonate.

9. A photographic silver halide emulsion in which the silver halide is dispersed in a hydrolyzed cellulose acetate containing from 20 to 26 per cent by weight of acetyl groups, said emulsion being sensitized with 2-methylmercaptobenzothiazole metho-p-toluenesulfonate.

10. A photographic silver halide emulsion in which the silver halide is dispersed in a hydrolyzed cellulose carboxylic ester containing from 19 to 33 per cent by weight of acyl groups, said emulsion being sensitized with at least one quaternary salt selected from the group consisting of those quaternary salts represented by the following general formula:



wherein D represents an o-arylene group of the benzene series containing from 6 to 8 carbon

9

atoms and which is devoid of nitro groups, R represents a primary alkyl group containing from 1 to 4 carbon atoms, R<sub>1</sub> represents an arylmercapto group containing from 6 to 8 carbon atoms and devoid of nitro groups, and X represents an anion.

11. A photographic silver halide emulsion in which the silver halide is dispersed in a hydrolyzed cellulose acetate containing from 19 to 33 per cent by weight of acetyl groups, said emulsion being sensitized with at least one quaternary salt selected from the group consisting of those quaternary salts represented by the following general formula:



where in D represents an o-arylene group of the benzene series containing from 6 to 8 carbon atoms and which is devoid of nitro groups, R represents a primary alkyl group containing from 1 to 4 carbon atoms, R<sub>1</sub> represents an arylmercapto group containing from 6 to 8 carbon atoms and devoid of nitro groups, and X represents an anion.

12. A photographic silver halide emulsion in which the silver halide is dispersed in a hydrolyzed cellulose acetate containing from 20 per cent to 26 per cent by weight of acetyl groups, said emulsion being sensitized with at least one quaternary salt selected from the group consisting of those quaternary salts represented by the following general formula:



10

wherein D represents an o-arylene group of the benzene series containing from 6 to 8 carbon atoms and which is devoid of nitro groups, R represents a primary alkyl group containing from 1 to 4 carbon atoms, R<sub>1</sub> represents an arylmercapto group containing from 6 to 8 carbon atoms and devoid of nitro groups, and X represents an anion.

13. A photographic silver halide emulsion in which the silver halide is dispersed in a hydrolyzed cellulose acetate containing from 20 per cent to 26 per cent by weight of acetyl groups, said emulsion being sensitized with 2-phenylmercaptobenzothiazole ethiodide.

15

BURT H. CARROLL.  
WILLIAM WEST.

## REFERENCES CITED

20 The following references are of record in the file of this patent:

## UNITED STATES PATENTS

| Number    | Name           | Date           |
|-----------|----------------|----------------|
| 2,110,491 | Salo           | Mar. 8, 1938   |
| 2,131,038 | Brooker et al. | Sept. 27, 1938 |
| 2,271,623 | Carroll        | Feb. 3, 1942   |
| 2,334,864 | Carroll et al. | Nov. 23, 1943  |

## FOREIGN PATENTS

| Number  | Country       | Date          |
|---------|---------------|---------------|
| 496,049 | Great Britain | Nov. 21, 1938 |

35

40